

Dec. 8, 1942.

R. W. PEAKES

2,304,137

PROTECTIVE GLOVE

Filed Dec. 15, 1932

FIG. 1



FIG. 2



FIG. 3



FIG. 4



Inventor

RALPH W. PEAKES

By Joseph A. O'Connell and  
Fred S. Lockwood  
attorneys

## UNITED STATES PATENT OFFICE

2,304,137

## PROTECTIVE GLOVE

Ralph W. Peakes, Edgewood Arsenal, Md., assign.  
or to Patrick J. Hurley, Secretary of War of the  
United States of America, and his successors  
in office

Application December 15, 1932, Serial No. 647,495

5 Claims. (Cl. 2—168)

(Granted under the act of March 3, 1883, as  
amended April 30, 1928; 370 O. G. 757)

The invention described herein may be manufactured and used by or for the Government for governmental purposes, without the payment to me of any royalty thereon.

This invention relates to the manufacture of protective gloves which are specially treated to protect the wearer thereof from the vesicant effect of various chemicals such as mustard gas.

It is well known that modern warfare involves the use of various gases which have more or less injurious effects upon the skin of those coming in contact therewith.

Many protective devices have been developed for the protection of persons exposed to these gases, either at the battlefield or in the factory producing the gases and filling the shells or grenades therewith.

Heretofore no practicable gloves have been available which afford complete protection to the hands of the wearer and yet have sufficient flexibility as not to materially interfere with the normal use of the hands.

The principal object of this invention therefore, is to provide a protective glove which is impermeable to injurious gases.

Another object of this invention is to provide a protective glove which is impermeable to injurious gases and which is sufficiently flexible to allow free use of the hand.

Another object of this invention is to provide a glove which fully protects the wearer's hand against vesicant gases while allowing free use of the hand, and which is durable in use.

Another object of this invention is to provide a glove formed of an inner liner which is impermeable to vesicant gases such as mustard gas, and an outer waterproof glove capable of withstanding the normal wear to which the glove is subjected and protecting the inner lining from mechanical injury and moisture.

A further object of this invention is to provide a glove formed of an inner liner and an outer glove as above described and which is not cumbersome nor stiff in use.

A further object of this invention is to provide a protective inner liner for gloves composed of a relatively light fabric treated to render the same impervious to vesicant gases. More specifically it is an object of this invention to provide a liner of this character treated with viscose latex, Cellophane, viscose compounds or similar protective materials.

These and other objects of this invention will be apparent from the following description and appended claims, it being understood that the

several necessary substances and compounds and the materials treated may be widely varied, the following description being by way of example only and without limiting the invention to the specific embodiments set forth.

Figure 1 is an elevation of the glove and impermeable lining, with a portion of the fabric and lining broken away.

Figure 2 is an enlarged section of the fabric partially separated from the coating.

Figure 3 is a similar section of a modified form.

Figure 4 is a section showing a seam of the lining, and the assembly with the outer glove.

One preferred embodiment of this invention is as follows. A relatively light and flexible fabric 1 such as cotton fabric, balloon cloth, or the like, is treated with a compound 2 to render it impermeable to mustard gas or similar gases. The compound used for this purpose is a cellulose derivative, such as viscose latex, Cellophane, or other viscose compounds. Excellent results have been obtained by the use of viscose-rubber latex as a coating.

The coating mixture 2 may be applied to the fabric in any approved manner. As one example, 2-ounce cotton fabric 3 lightly coated with rubber 4 on one side, to which a thin coating of viscose and rubber latex 5 plasticized with glycerine is attached by a thin layer of glue 6 may be used. However, greater flexibility of the glove may be obtained by directly coating the fabric with viscose or viscose-rubber latex plasticized with glycerine, without the initial light coat of rubber and without the addition of glue. This preferred embodiment gives ample protection against vesicant gases and liquids and allows full freedom of the hand.

The coated fabric is then cut to the shape of a glove, and the seams carefully sewed. The sewed seams of these inner gloves are next rendered resistant to mustard gas or similar gases by covering them with rubberized tape 7, as seen in Figure 4. A preferred method, however, is to coat the seams with rubber latex or cellulose nitrate or cellulose acetate composition, preferably by spraying.

The inner glove made as described is then inserted into an outer wear-resistant glove of any suitable type such as cotton fabric glove 8 coated with a plasticized cellulose nitrate composition for example, or a drying oil composition, or leather or canvas glove. Preferably the coated side of the liner is placed next to the inner side of the outer glove. Prior to assembly of the inner and outer

gloves, however, both gloves are impregnated with glycerine to preserve flexibility.

The inner liner is then securely fastened within the outer glove by stitching 9 along the top of the glove and also around the opening for the hand.

Preferably the outer glove is waterproofed in any approved manner to prevent passage of moisture which might injure the impregnated liner.

Protective gloves made in accordance with the present invention afford protection against penetration by liquid mustard for fifteen hours. Furthermore, the durability of these gloves is such that they will outlast several pairs of cellulose nitrate-rape seed oil coated gloves previously in use, and are more flexible and comfortable.

Tests have demonstrated that gloves made in accordance with this invention wherein a vesicant chemical resistant inner liner is secured at spaced points within a wear and moisture resistant outer glove, afford excellent protection. This type of assembly results in a glove with a mustard gas resistance many times greater than the sum of the mustard resistance value of the constituent layers of the material, due to the main portion of the layers being unattached and slightly spaced from one another. The flexibility of this glove is also greater than that obtained by the same layers joined together throughout. The multiple layer construction allows the utilization of many materials which otherwise have proved to be valueless where flexibility, gas resistance, and durability are essential requirements.

It will be seen therefore that the present invention provides gloves which afford full protection against injurious gases for long periods of time, are extremely durable, and allow complete flexibility of the hand.

While I have described the preferred embodiment of my invention, I wish it to be understood that the invention is not limited to the precise ingredients and steps described herein by way of illustration, as it will be apparent that many changes in variations may be made without departing from the spirit of the invention or the scope of the appended claims.

I claim:

1. A glove comprising an inner liner composed of fabric treated to render it impervious to vesicant gases, and an outer glove composed of wear-resisting material, said liner and outer glove being secured together to maintain their assembly but having their main surfaces unattached, said inner liner comprising a light cotton fabric having a coating of rubber, and a second coating of viscose-rubber latex.

2. A glove comprising an inner liner composed of fabric coated with a thin layer of viscose-rubber latex plasticized with glycerine to render the same impervious to vesicant gases, and an outer glove composed of wear-resisting liquid-proof material, said liner and outer glove being secured in assembled relation with their main surfaces unattached.

3. A glove for protection against chemical warfare agents such as mustard gas comprising an inner liner composed of light flexible fabric coated with one of the compounds consisting of viscose, or other cellulose derivative, and an outer glove of wear-resisting material, said liner and outer glove being attached only at widely spaced extremities thereof to thereby provide an air space between the main portions.

4. A glove for protection of the wearer against mustard gas and other vesicant chemical agents comprising an inner glove formed of light flexible cotton fabric having an impervious coating of viscose and rubber latex on the inner surface, and an outer glove of heavy waterproof wear-resistant material, said inner and outer gloves being assembled and secured together at widely spaced portions, whereby an air space is maintained between the inner and outer gloves to provide additional protection against vesicants.

5. A glove for protection against chemical warfare agents such as mustard gas comprising an inner liner formed of light flexible fabric treated with a mustard gas resistant material, and an outer glove of wear-resisting material, said liner and outer glove being attached only at widely spaced extremities thereof to thereby provide an air space between the main portions.

RALPH W. PEAKES.